

Nov. 20, 1923.

1,474,653

K. L. TORNO

TILE AND METHOD OF MANUFACTURING THE SAME

Filed Oct. 4, 1921

*Fig. 1.*



*Fig. 2.*



*Fig. 3.*



*Fig. 4.*



INVENTOR  
KARL L. TORNO  
BY ATTORNEY

*Lincoln Johnson*

Patented Nov. 20, 1923.

1,474,653

# UNITED STATES PATENT OFFICE.

KARL L. TORNO, OF BERKELEY, CALIFORNIA.

## TILE AND METHOD OF MANUFACTURING THE SAME.

Application filed October 4, 1921. Serial No. 505,252.

To all whom it may concern:

Be it known that I, KARL L. TORNO, a subject of the Kingdom of Sweden, having received my first papers of citizenship in the 5 United States of America, and a resident of the city of Berkeley, county of Alameda, State of California, have made a new and useful invention—to wit, Tiles and Methods of Manufacturing the Same; and I do hereby declare the following to be a full, clear, 10 concise, and exact description of the same.

This invention relates particularly to a decorative finish for porous surfaces.

The principal object of this invention relates to the method of applying a decorative facing to porous surfaces, particularly tiles, which when finished will have the appearance of a burned or heat treated article. A still further object relates to the method of 20 applying a decorative facing to tiles and the like, whereby it becomes possible to tint or color the said tiles and the like in any desirable manner and to any desirable extent. Other objects and advantages will appear as 25 this description progresses.

In this specification and the annexed drawings, the invention is illustrated in the form considered to be the best, but it is to be understood that the invention is not limited to such form, because it may be embodied in other forms; and it is also to be understood that in and by the claims following the description, it is desired to cover the invention in whatsoever form it may be embodied.

In the accompanying one sheet of drawings:

Fig. 1 illustrates a perspective of a tile manufactured in accordance with my invention.

Fig. 2 represents a cross section of a tile manufactured in accordance with the initial step of my invention.

Fig. 3 represents a cross section through a tile treated in accordance with the second step of my invention.

Fig. 4 is a cross section through a tile being treated in accordance with the final step of my invention.

The limitations of a patent drawing convey no conception of the artistic merit of the invention and it is submitted merely to illustrate the structure.

The interiors of homes, residences and the like are rendered unusually artistic by installing ornamental mantel pieces of tile

around fire places, providing tiled floors and tiled wainscoting after the manner of residences representative of early periods of architecture abroad. The tile or porous material used is generally formed from a suitable clay or earthen material in a plastic form colored in any predetermined manner and then placed in an oven and baked or heat treated until the mass hardens. This process is unusually long and tedious and is objectionable in that the desired final color schemes of the tile cannot always be assured with absolute accuracy by reason of the chemical change resulting through the application of heat to the plastic material. Where certain of the baked tiles are discolored and do not blend with the greater portion of the tile treated, the same must be rejected, thereby entailing a loss of time and material to the manufacturer. Furthermore where it is desired to have an ornamental design embodied in the usual type of baked tile it becomes necessary to stamp the same with a specially prepared die which as a result, lacks artistic merit. The usual baked tile is likewise very close grained in texture so that binding mortar will not adhere as readily as with tiles constructed in accordance with my invention.

The tiles utilized in the practice of my invention are formed from an aggregate of moistened sand, cement and gravel which is permitted to set until the desired degree of hardness has been attained.

In applying the decorative coating, or facing to the surface of the tile, a plurality of tiles are laid in a single layer on a suitable surface so that the edges of all tiles are in contact. With a brush or other suitable means I apply a cementitious fluid to the exposed surfaces and edges of the tiles and work the same well into the said tiles, as shown in Fig. 1. The said cementitious fluid is preferably formed from a mixture of water and either a powdered plaster, cement or magnesite worked to a creamy consistency. The consistency of the said cementitious mixture is such that when applied to the surface of the tiles evenly it assumes the same configuration as the surface underneath. This surface texture if desired, can be changed by agitating the tiles which settles the cementitious material in the mixture to the bottom and causes the upper portion of the mixture to assume a flat smooth finish. As a usual matter it is not desirable

to agitate the tile in view of the fact that such tiles do not reach the same degree of perfection as those treated in the following manner.

- 5 In the second step of my process, as shown in Fig. 3, I sprinkle or apply powdered coloring material, of any desirable nature according to the color or finish desired, onto the moist exposed face of the fluid applied to the tile. In order to achieve the effects embodied in burned tiles, powdered coloring matter would be applied irregularly in amount and position on the tile, leaving a somewhat mottled appearance.
- 10 15 A stippling brush or other similar tamping means, of which the resilient ends would be curled over to provide a softened body, would be first moistened and then applied to the combined cementitious fluid and coloring material to thoroughly intermix the same, working said coloring material into and throughout the entire mass of the cementitious mixture. The stippling brush would then be cleansed of such coloring material as might have adhered to it around the ends and it would be remoistened after which portions of the tile not so fully treated with the coloring material would be tamped after the manner of the first stippled portion.
- 20 25 30 35 40 45 After stippling or tamping the entire mottled surface of the tiles with the moistened brush so that the resemblance to a baked tile would be clearly effective, the tiles would then be placed on separate trays and permitted to dry or harden. The facing or decorative surfaces applied to the tiles being formed from a cement or magnesite base would assure the hardness of a dried cement or dried magnesite and would be thus impervious to the effects of moisture or any other elements.

After the facing on the tiles has set, the same might be polished or buffed to present a smooth, shining surface or this last named operation omitted if a rough finish be desired. In the completed condition, my tiles may be used in lieu of baked tiles in all instances where such tiles might be used. The advantages of using tiles constructed in ac-

cordance with my invention are first, that the same may be produced in about one-quarter the time, manufactured at about one-third of the cost and sold for about one-half the selling price of baked tiles.

Where it is desired to have a specially prepared decorative tile with an ornamental design embodied therein, similar to baked stamped tiles, I first apply the cementitious fluid mixture to the tile and then with suitable portions of differently colored cementitious mixture added to the first mixture on the tile produce artistic picture effects such as landscapes, marine views, trees, flowers and the like. These colored mixtures would correspond to the powdered coloring material, applied to the tiles as first described, but the addition of two or more colors superimposed one on the other would result in any number of different designs and effects according to the manner of application.

Having thus described this invention what I claim and desire to secure by Letters Patent is:—

1. The method of finishing porous surfaces consisting in applying a cementitious fluid to said surface; adding coloring matter to said surface, and stippling said coloring matter and fluid.
2. The method of finishing porous surfaces consisting in applying a cementitious fluid to said surface; adding coloring matter of a cementitious nature to said surface, stippling said coloring matter and fluid and permitting the same to harden.
3. The method of finishing tiles comprising coating said tiles with a cementitious fluid; sprinkling powdered coloring matter of a cementitious nature on to said fluid coating; stippling said coloring matter into said fluid surface and permitting the mixture to harden.

In testimony whereof, I have hereunto set my hand at San Francisco, California, this 26th day of Sept. 1921.

KARL L. TORNO.

In presence of—  
LINCOLN V. JOHNSON.